

April 30, 1935.

C. B. HEMMING ET AL

1,999,413

METHOD OF DECORATING SURFACES

Filed Aug. 12, 1931



Fig. 1



Fig. 2

INVENTORS

Charles B. Hemming  
Earl C. Pitman  
BY

J. W. Biddle Jr.  
ATTORNEY.

## UNITED STATES PATENT OFFICE

1,999,413

## METHOD OF DECORATING SURFACES

Charles B. Hemming, Parlin, and Earle C. Pittman, Princeton, N. J., assignors to E. I. du Pont de Nemours & Company, Wilmington, Del., a corporation of Delaware

Application August 12, 1931, Serial No. 556,606

7 Claims. (Cl. 41—33)

This invention relates to a method of decorating surfaces, and more particularly to a method employing the use of decalcomanias and to the product obtained thereby.

5 The present invention involves the use of the common type of decalcomania, in which a sheet of paper or similar material is first coated with a water soluble size, usually a gum, and then the decalcomania is lithographed on the coated surface with the back side of the decalcomania up. This type of decalcomania is usually applied by coating the back side of the decalcomania with a water insoluble size, usually of the varnish type, and then applying the whole to the surface to be decorated when the coating has reached a tacky state. The decalcomania is then rolled under pressure and the surface subsequently washed with water to remove the paper backing and water soluble size. As a final step, the surface is coated with a clear top coat composition to protect the decalcomania.

A modification of this type of decalcomania is the so-called "duplex decalcomania", in which the decalcomania is lithographed on to thin, 25 translucent paper in place of the usual thick white paper. As the combination is rather fragile, the whole is mounted on thicker paper by means of a very light coat of a gummy adhesive. This type of decalcomania is used in the same manner as the first type, except that after 30 the decalcomania is applied to the surface to be decorated the thick sheet of paper is stripped off without washing, the second thin sheet being removed by washing as in the ordinary decalcomania. This type of decalcomania is advantageous due to the fact that the thick sheet may be waterproof, obviously impossible in the ordinary decalcomania, and also the thin sheet may be readily removed by washing, thus reducing 35 the danger of damaging the design layers of delicate decalcomanias.

40 There are other types of decalcomanias employing the same basic principles, among which may be mentioned the recently developed thin photo film decalcomania.

45 All of these decalcomanias are far from satisfactory, the basic difficulty usually being due to the fact that the design layer of the decalcomania itself is not anchored securely to the surface to be coated and, as a result, the detail of the design layer is likely to be blurred while being applied, and lifting and poor wearing qualities frequently are characteristic of surfaces decorated in this manner.

50 An object of the present invention is to provide a method whereby the decalcomania is firmly anchored to the surface to be decorated so that the above difficulties are avoided. Other advantages will be apparent from the description 55 of the invention given hereinafter.

The above objects are accomplished according to the present invention by first applying to the surface to be decorated a ground coat adapted to harden on application of heat, then allowing this ground coat to dry until it reaches a tacky state, then applying the decalcomania, using pressure and a somewhat elevated temperature. Preferably, the decalcomania is applied by means of a hydraulic press. After application of the decalcomania the surface is washed to remove the paper or similar backing of the decalcomania and the water soluble size, and the coated surface is then baked until hard. Subsequently, a clear top coat is applied to the decorated surface and this is preferably also a composition adapted to harden upon the application of heat. If this type of clear top coat is employed, the surface is again baked to harden the top coat.

5 One embodiment of the invention is illustrated in the accompanying drawing in which Fig. 1 shows a sectional view and Fig. 2 an elevation, with parts broken away for clarity, of a metal sheet decorated as described in the example below.

20 The following example is given to illustrate a preferred method of carrying out the present invention:

25 Example 1.—A pigmented ground coat was applied by roller coating, directly to a clean metal surface which had been scuffed, and air dried for approximately 1 hour, at the end of which time the coat was slightly tacky. The composition of this ground coat was as follows:

|                                                        | Per cent |
|--------------------------------------------------------|----------|
| Titanium oxide                                         | 34.0     |
| *Modified polyhydric alcohol-polybasic acid type resin | 44.8     |
| Petroleum solvent naphtha                              | 5.8      |
| Heavy petroleum naphtha                                | 6.0      |
| Hi-flash naphtha                                       | 3.1      |
| Mineral spirits                                        | 6.3      |
|                                                        | 100.0    |

45 \*Modified polyhydric alcohol-polybasic acid type resin.

|                    | Per cent |
|--------------------|----------|
| Phthalic anhydride | 46.30    |
| Glycerol           | 21.24    |
| Linseed oil acids  | 30.97    |
| Glycol             | 1.49     |
|                    | 100.00   |

55 After the specified drying period the decalcomania was applied by laying it on the slightly tacky ground coat, placing the whole on a hydraulic press and applying a pressure of 900 pounds per square inch, the plates of the press 60

being heated to 100° C. Pressure was maintained for a period of one minute.

The piece of metal being decorated was then removed, cooled, and the paper backing and the water soluble size of the decalcomania entirely removed by a thorough washing with water. The article was then baked one hour at 82° C. After the bake, a clear protective top coat was applied by roller coating and the article given a final bake at 82° C. for one hour. The clear top coat had the following composition:

|                                                                | Per cent |
|----------------------------------------------------------------|----------|
| Polyhydric alcohol-polybasic acid type resin (described above) | 30.0     |
| 15 Blown rapeseed oil                                          | 1.0      |
| Hi-flash naphtha                                               | 64.4     |
| 5% cobalt linoleate solution in turpentine                     | 4.4      |
| Oil of cloves                                                  | 0.2      |
|                                                                | <hr/>    |
| 20                                                             | 100.0    |

The above example gives a very specific method of carrying out the present invention and may be modified greatly. It has been found that 25 the following represent approximately the operative limits of the process:—

|                                          |                         |
|------------------------------------------|-------------------------|
| Decalcomania anchoring pressure          | 40# to 900# per sq. in. |
| 30 Decalcomania anchoring temperature    | 70° C. to 150° C.       |
| Decalcomania anchoring time              | .05 to 5.0 minutes      |
| Ground coat and final baking temperature | 60° C. to 150° C.       |
| Ground coat and final baking times       | 8 hours to 20 minutes   |

It will be understood, however, that the invention can be carried out, and may be carried out, outside of these limits under special circumstances. As will be apparent to those skilled in the art, the baking period will vary inversely with respect to the baking temperatures given above.

45 It is preferred to apply the ground coat and the clear top coat by roller coating, although same may be applied by dipping, brushing, spraying, or other methods used in the art.

The method of decorating is obviously not only 50 applicable to metal, but to many other surfaces, such as wallboard, linoleum, and similar compositions of matter.

The type of ground coat composition used in this method is of great importance and must be 55 such that it gives a film that will harden upon application of heat. By this is meant that the ground coat composition must be such that the application of heat will cause oxidation, polymerization, condensation or similar change to 60 give both a hard and inert film, as contrasted with compositions that merely dry through evaporation of solvents, such as nitrocellulose lacquers. Synthetic resin compositions are particularly suitable for the ground coat composition, for example, polyhydric alcohol-polybasic acid 65 "glyptal" type resin compositions and compositions employing phenol-formaldehyde resins, urea-formaldehyde resins, and the like. The oil type varnishes are also suitable for this purpose, although not as preferable where a metallic surface is to be decorated, as usually a primer coat 70 must first be applied to the metal to secure adequate adhesion of the oil varnish. With the synthetic resin compositions excellent adhesion is

obtained without the use of a primer coat. As will be apparent to those skilled in the art, the particular formula to be used can be widely varied. Various diluents, softeners, solvents, and pigments, and combinations thereof may be employed, the main consideration being that a composition of the "hardening" type disclosed is used.

The following formula is given to illustrate a typical oil type varnish suitable for use as the ground coat according to the present invention. The particular formula is well adapted for a ground coat where a walnut grain effect is desired on a surface:

| Walnut graining ground         | Percent |
|--------------------------------|---------|
| *Varnish base                  | 37.9    |
| Pigments                       | 52.2    |
| Lead-manganese drier solution  | 3.0     |
| Mineral spirits                | 2.7     |
| Solvenol (turpentine fraction) | 4.2     |
|                                | <hr/>   |
|                                | 100.0   |

\*Varnish base:

| Copal                          | Percent |
|--------------------------------|---------|
| China-wood oil                 | 13.7    |
| Linseed oil                    | 15.0    |
| Mineral spirits                | 10.5    |
| Solvenol (turpentine fraction) | 53.7    |
|                                | <hr/>   |
|                                | 7.1     |
|                                | 30      |

100.0

The pigments for this formula consist of:

|                            |    |
|----------------------------|----|
| Ferrite yellow dark orange | 35 |
| Lithopone                  |    |
| Chrome yellow medium       |    |
| Whiting                    |    |
| Cosmic black               |    |
| Red oxide                  |    |

In the manufacture of this finish, the pigments are ground in the varnish base. The other ingredients specified above are added in the final mixing cycle.

The composition can be widely varied, as will be understood by those skilled in the art. The varnish may comprise a combination of China-wood oil and linseed oil, with or without resins, and with a wide variety of solvents, diluents, driers, and pigments.

Regardless of whether a synthetic resin type ground coat or an oil varnish ground coat is used, the ground coat is allowed to dry until substantially all of the volatile solvents therein have evaporated before applying the decalcomania. In either type of ground coat a tacky film will be left after the volatile solvents have evaporated.

The composition of the clear top coat may be varied even more widely than the ground coat. Any composition that will give a clear film of satisfactory durability may be employed, although it is preferred to use a synthetic resin composition that will harden on heating so that by a final bake a product of great durability is obtained. However, cellulose derivative coating compositions and other coating compositions which dry simply through evaporation of the solvent constituent may be employed. Since the ground coat will have already been baked and thereby hardened prior to application of the clear top coat and become substantially insoluble in coating composition solvents, any known solvent mixture may be used in the top coat without danger of lifting or other harmful effects that would result if the

ground coat were subject to attack by the solvents in the clear coat. If desired, the clear top coat may be omitted, although it is preferred to have a protective coat over the decalcomania.

- 5 It is believed that the greatly improved anchorage of the design layer of the decalcomania according to the present invention is due to the use of a ground coat composition adapted to harden on application of heat, and the application of 10 the decalcomania with heat and pressure to the coated surface. The decalcomania is forced down into the ground coat, which affords a good anchorage while the backing of the decalcomania is removed by washing and the subsequent baking 15 and hardening of the ground coat effects a lasting anchorage of unexpected strength.

The particular construction of the decalcomania forms no part of the present invention, except that it is necessary to have the decalcomania manufactured with its front side in contact with the sheet of paper, or other backing used. The term "decalcomania" is used throughout to include only this type of decalcomania. The term "design layer" employed in the claims is 25 used to define the decorative layer which, together with the paper backing and sizing, forms the decalcomania. Where a "duplex" decalcomania of this type is used, obviously the thick sheet of paper backing must be stripped off dry 30 before the washing step.

The decalcomania can be applied to the tacky ground coat in a variety of ways, such as by roller, hydraulic press, etc., as long as some pressure is applied in forcing it down. It is preferred to place 35 the article to be decorated between the plates of a hydraulic press and then to apply the decalcomania with heat and pressure within the limits above specified. By this means delicate decalcomanias can be applied without the slightest blur or imperfection.

40 The method of the present invention may be successfully utilized in the manufacture of metal furniture, automobile dash boards and moldings, in tin decorating, in the production of wall tile 45 involving decalcomania transfers, linoleum desk tops, et cetera.

An important advantage of the present method over methods heretofore known for applying decalcomanias, is the greatly improved anchorage 50 of the decalcomania to the surface to be decorated. Lifting, which heretofore had generally been encountered in surfaces decorated with decalcomanias is entirely eliminated. Furthermore, decalcomanias applied according to the 55 present invention are so firmly anchored that they are able to withstand severe forming operations upon the decorated surface without peeling or cracking at the points under stress. This latter characteristic is of great advantage in manufacturing dash boards and other metal articles which 60 must be subjected to a forming operation.

The present method is extremely simple and easily carried out in commercial production. Surfaces such as clean scuffed auto body steel, or 65 clean scuffed black iron, are suitable to be decorated, and the close control and extreme precaution which was necessary in the older methods for applying decalcomanias are eliminated in the present method, where satisfactory results may 70 be obtained with only normal care.

A particularly satisfactory and improved decorated surface is obtained where both the ground coat and clear top coat are synthetic resin compositions of the "glyptal" type. A hard surface 75

of great durability and better appearance, as well as materially improved adhesion, is obtained in this manner.

By the term "composition adapted to harden upon application of heat", as used in the appended claims, is meant a composition that will harden and become substantially inert upon application of heat, to various coating composition solvents.

As many apparently widely different embodiments of this invention may be made without departing from the spirit and scope thereof, it is to be understood that we do not limit ourselves to the specific embodiments thereof except as defined in the appended claims.

We claim:

1. Method of decorating a surface comprising applying a ground coat composition thereto adapted to harden upon application of heat, drying the coated surface until tacky, applying a 20 decalcomania to the coated surface at a temperature of 70-150° C. and pressure of 40-900 pounds per square inch, washing the surface to remove the backing and sizing of the decalcomania, baking the coated surface until hard, and applying over the coated surface a clear top coat.

2. Method of decorating a surface comprising applying a polyhydric alcohol-polybasic acid resin ground coat composition thereto adapted to harden upon application of heat, drying the coated surface until tacky, applying a decalcomania to the coated surface with pressure, washing the surface to remove the backing and sizing of the decalcomania, and baking the coated surface until hard.

3. Method of decorating a surface comprising applying a polyhydric alcohol-polybasic acid resin ground coat composition thereto adapted to harden upon application of heat, drying the coated surface until tacky, applying a decalcomania to the coated surface with heat and pressure, washing the surface to remove the backing and sizing of the decalcomania, baking the coated surface until hard, and applying over the coated surface a clear top coat.

4. Method of decorating a surface comprising applying a polyhydric alcohol-polybasic acid resin ground coat composition thereto adapted to harden upon application of heat, drying the coated surface until tacky, applying a decalcomania to the coated surface with heat and pressure, washing the surface to remove the backing and sizing of the decalcomania, baking the coated surface until hard, applying over the coated surface a polyhydric alcohol-polybasic acid resin clear top coat adapted to harden upon application of heat, and again baking the coated surface to harden the top coat.

5. Method of decorating a surface comprising applying a polyhydric alcohol-polybasic acid resin ground coat composition thereto adapted to harden upon application of heat, drying the coated surface until tacky, applying a decalcomania to the coated surface at a temperature of 70-150° C. and with a pressure of 40-900 pounds per square inch, washing the surface to remove the backing and sizing of the decalcomania, baking the coated surface until hard, applying over the coated surface a polyhydric alcohol-polybasic acid resin clear top coat adapted to harden upon application of heat, and again baking the coated surface to harden the top coat.

6. An article comprising a base having a hard

baked ground coat comprising a polyhydric alcohol-polybasic acid resin, a design layer over said ground coat, and a hard, baked, clear top coat comprising a polyhydric alcohol-polybasic acid resin applied over said design layer.

7. An article comprising a sheet of metal having a hard baked ground coat comprising a poly-

hydric alcohol-polybasic acid resin, a design layer over said ground coat, and a hard, baked, clear top coat comprising a polyhydric alcohol-polybasic acid resin applied over said design layer.

CHARLES B. HEMMING.  
EARLE C. PITTMAN.